

(No Model.)

C. M. BALL & S. NORTON.

PROCESS OF SEPARATING ORES BY MAGNETISM.

No. 404,332.

Patented May 28, 1889.



WITNESSES:

*C. M. Ball*  
*J. C. Sneath*

Clinton M. Ball } INVENTORS  
Sheldon Norton }

BY  
*W. F. G. Worthington,*  
ATTORNEYS

# UNITED STATES PATENT OFFICE.

CLINTON M. BALL, OF TROY, AND SHELDON NORTON, OF WEST TROY, AS-SIGNORS OF ONE-THIRD TO ALEXANDER T. PORTER, OF WEST TROY, NEW YORK.

## PROCESS OF SEPARATING ORES BY MAGNETISM.

SPECIFICATION forming part of Letters Patent No. 404,332, dated May 28, 1889.

Application filed September 26, 1888. Serial No. 286,398. (No model.)

*To all whom it may concern:*

Be it known that we, CLINTON M. BALL, of Troy, in the county of Rensselaer, and SHELDON NORTON, of West Troy, in the county of 5 Albany, and State of New York, both citizens of the United States, have invented certain new and useful Improvements in Processes of Separating Ores; and we do hereby declare the following to be a full, clear, and exact de- 10 scription of the invention, such as will enable others skilled in the art to which it appertains to make and use the same.

This invention relates to a novel method or process of separating magnetic ores from the 15 impurities with which they are generally found associated, such as phosphorus, sulphur in the form of pyrites, &c.

Briefly, the invention consists in forcibly causing the tumbling or rolling of the particles of crushed ore through a compound magnetic field of alternating polarity with or without the application of a current of air; and the invention further consists in the specific process and steps, substantially as hereinafter fully described and claimed.

In carrying out our process it is necessary to use some form of apparatus, and we illustrate the invention by means of an improved form of magnetic separator, but desire here 30 to state that we do not herein claim any apparatus, as such forms the subject-matter of another application filed by us October 3, 1888, Serial No. 287,329.

In the drawings, Figure 1 is a vertical section of a separating apparatus embodying the features of the present invention, and Fig. 2 illustrates diagrammatically the principle upon which our invention is based.

We construct the hopper 1, having an adjustable gate, with the distributing-edge 2, adapted to spread the ore and gangue uniformly and to an even depth over an inclined apron, 3, which feeds into a vertical chute, 4, whose lower end is connected to the inlet of 45 a rotary fan or blower, 5, which may be conveniently operated from the counter-shaft 14 by the belt 6 and pulley 7. Situated on the frame-work of the structure are the two parallel shafts 8 9, and these carry the drums 10 50 and 11, over which is passed an endless belt,

12, or screen, of material which is preferably non-magnetic, drum 11 being driven positively by means of a belt connected with any suitable source of power. Both or either of the ends of the apparatus between the drums 55 10 and 11 and the face of the inclined apron 3 may be open to the atmosphere, so that in the operation of the blower 5 currents of air are induced at these points and deflected downwardly into chute 4, as indicated by arrows in the figure. In the space between the drums 10 and 11, I place a series of magnets,  $M M^2 M^3 M^4$ , &c., and these magnets may be either permanent or electro magnets, and they are so arranged as to have their free 60 poles in close proximity to the inner face of the belt 12, next the inclined apron 3. The free poles are arranged in alternation as to polarity—that is, if the first pole is north the second is south, the third north, the fourth 70 south, and so on throughout the series, which may be of any desired number.

The operation will be as follows: The ore and gangue passing down the apron 3 come within the attractive influence of the first pole 75 of the magnetic system and all magnetic particles contained in the body of ore are immediately attracted and held against the moving belt 12, which on this side is moving downwardly, as indicated by the large arrow. All 80 the magnetic particles are attracted first to the first pole; but as the belt compels them to move forward toward the second pole their positions are reversed, and, leaving the second pole for the third pole, their positions are 85 again reversed, and so on past the series of magnets in succession, so that all the magnetic particles are not merely caused to adhere against the face of the belt, but as they pass along are compelled to, as it were, tumble or turn end for end, and in this manner are very thoroughly agitated and their friction upon one another and upon the belt, along with the mechanical agitation effected by the alternations of magnetic polarity, result in a 90 most thorough cleansing of the magnetic particles from all dust or other impurities which would otherwise cling to them. The peculiar action upon the magnetic particles is graphically illustrated in Fig. 2, where, for the pur- 100

pose of clearness, a single particle is shown in its successive positions as it travels past the alternating poles of the magnetic system, the particle being exaggerated in size in order to make the action clear. On inspection of this figure it will be observed that as the particle first approaches the magnetic system it becomes polarized by induction and one end becomes attracted more strongly than the other, owing to this induced polarity, and as it passes such pole it stands on end, in accordance with the well-known phenomena of the lines of force in magnetic substances. As it is carried forcibly past this pole its outer and free end tends toward the next pole of the magnetic field, and midway between the two the position of the particle is parallel with the belt, and when it reaches the second magnetic pole it again stands on end, but this time on the opposite end from that on which it stood at the last stage, and so on throughout the entire series of poles of the compound magnetic field, the magnetic particle is drawn by the belt and at the same time compelled by the magnetic attractions to tumble end over end, as it were, a sufficient number of times to absolutely cleanse it of all foreign substances and dust which might be clinging to its exterior. As the gangue approaches the chute 4 most of the unmagnetizable portions fall into the chute and are carried away by the current of air produced by the blower 5, and as a final step toward perfectly cleaning the magnetized particles which are now past the chute and are ready to be delivered, the induced current of air upwardly past the lower end of apron 3 has the effect of blowing away the last traces of dust and all other impurities which may possibly be still clinging to the particles of magnetic ore, after which the belt carries them

outside the magnetic field, and as they are no longer attracted they fall on the lower end of apron 3, and thus are not merely separated from the gangue, but also perfectly cleaned. 45

We have shown and described a particular manner of utilizing a blast of air; but we do not confine ourselves to the particular mode indicated above, as the same is subject to modification, as are also all the parts of the 50 apparatus herein described; but as the same do not form any portion of the invention embraced by this application we do not herein attempt to describe any such modifications, as such would be modifications of form of apparatus, and will be referred to in the other application accompanying this.

We claim as our invention—

1. The process of separating iron or its ore from impurities, consisting in forcing it in a 60 state of division past a succession of two or more magnetic poles of alternating polarity, whereby the particles are forcibly caused to tumble or rotate end for end.

2. The process of separating iron or its ore 65 from impurities, consisting in forcing it in a state of division past a succession of two or more magnetic poles of alternating polarity, while interposing a non-magnetic screen between the ore and the poles. 70

3. The process of separating iron or its ore from impurities, consisting in forcing it in a divided state past a succession of magnetic poles of alternating polarity, while subjecting the material to the action of a current of air. 75

In testimony whereof we affix our signatures in presence of two witnesses.

CLINTON M. BALL.  
SHELDON NORTON.

Witnesses:

FRED E. OOTHOUT,  
LEWIS H. McDONALD.